

No. 882,637.

PATENTED MAR. 24, 1908.

J. B. HUFFARD.

PROCESS OF PRODUCING SLAG FREE FERROCHROMIUM.

APPLICATION FILED JULY 10, 1907.



Witnesses:

John B. Huffard  
Chas. H. Potter.

Inventor:

John B. Huffard,  
Bymer & Fawcett,  
Att'y's.

# UNITED STATES PATENT OFFICE.

JOHN B. HUFFARD, OF FERRIS, WEST VIRGINIA, ASSIGNOR TO ELECTRO-METALLURGICAL COMPANY, OF CHICAGO, ILLINOIS, A CORPORATION OF WEST VIRGINIA.

## PROCESS OF PRODUCING SLAG-FREE FERROCHROMIUM.

No. 882,637.

Specification of Letters Patent. Patented March 24, 1908.

Application filed July 10, 1907. Serial No. 383,059.

*To all whom it may concern:*

Be it known that I, JOHN B. HUFFARD, a citizen of the United States, residing at Ferris, in the county of Fayette and State of 5 West Virginia, have invented certain new and useful Improvements in Processes of Producing Slag-Free Ferrochromium, of which the following is a specification.

The slags produced in the manufacture of 10 ferrochromium in an electric furnace are highly basic and infusible, containing oxids of calcium, magnesium, chromium and aluminium in such proportions that the melting point of the slag is higher than that of the 15 alloy.

In order to effect a separation of the slag and alloy, it is customary to tap the entire 20 contents of the electric furnace into a pot having a refractory lining, allow it to remain therein until the slag and alloy have partially 25 solidified, and then dump the mass into water to complete the cooling. Slag and adherent fused portions of the pot-lining are then broken and chipped away from the 30 alloy by pneumatic hammers or hand tools. This process is expensive and unsatisfactory as the slag is very hard and adheres so tenaciously that some of it remains and is carried by the alloy into the molten steel to which the 35 ferrochromium is added, to the injury of the finished product.

The present invention is an improved process of obtaining clean ferrochromium by effectively separating the molten alloy and 40 slag. According to this process the ferrochromium and slag are tapped from the electric furnace into a pot having a lining. The heavier alloy subsides and the superincumbent slag quickly solidifies or stiffens, while

the metal beneath remains molten. The tap-hole in the bottom of the pot is then opened 45 and the molten ferrochromium is run out into the ingot mold. The solid body of slag is then discharged from the pot, which is relined for further use.

Suitable apparatus is shown in the accompanying drawing, in which the figure is a transverse vertical section of the pot and ingot mold.

The cast iron pot 1, mounted on wheels 2, 50 has a thin fire-clay lining 3. In the lower end of the pot is a taphole 4 normally closed by a refractory plug. Beneath the pot is an ingot mold 5. A body of solidified or stiffened slag 6 is shown in the upper half of the 55 pot, while the molten ferrochromium 7 is flowing through the open taphole into the mold.

I claim:

1. The process of producing metals free 60 from slags of relatively-high melting-points, which consists in discharging the molten metal and slag into a vessel, allowing the metal and slag to stratify and the slag to solidify, and separating the molten metal 65 from the solid slag.

2. The process of producing slag-free ferrochromium, which consists in discharging the molten ferrochromium and slag into a vessel, 70 allowing the alloy and slag to stratify and the slag to solidify, and separating the molten alloy from the solid slag.

In testimony whereof, I affix my signature in presence of two witnesses.

JOHN B. HUFFARD.

Witnesses:

J. R. EDMANDS,  
GEO. T. LANCASTER.